

## UNITED STATES PATENT OFFICE

2,308,065

## METHOD OF MAKING EXPANSION JOINTS

Clarence R. Eckert, Englewood, N. J., assignor to  
The Celotex Corporation, Chicago, Ill., a cor-  
poration of Delaware

No Drawing. Application December 10, 1938,  
Serial No. 244,921

6 Claims. (Cl. 117—140)

This invention relates to improvements in the structural building arts, and particularly relates to expansion joint material used in connection with all kinds of structures, particularly concrete structures such as bridges, highways and the like.

Due to the fact that structures of this character have a tendency to expand and contract with temperature changes, it is common practice to interpose expansion joints at predetermined intervals in the structures. Such expansion joints must of necessity have certain resilient qualities and at the same time must be enduring and not readily affected by moisture or be subject to deterioration when exposed to the elements. A practical joint should also be one which is capable of being handled and put into place in an efficient and workmanlike style without an exceptional amount of skilled effort. Furthermore, the joint material must be one which can be produced at a fairly reasonable cost.

Heretofore, expansion joint materials of this character have been produced and sold, but most of them have one or more objections in that some are subject to rapid deterioration, and are not essentially waterproof, and are also somewhat hard to install under the varying conditions encountered. Prior to my invention, a further objection to the expansion joints previously manufactured has been that they have been made with volatile solvents with the incumbent hazards of fires and explosion.

An object of my invention is to produce a highly efficient joint of standard building material so arranged and treated as to afford all the advantages desired in joints of that character and eliminating to a great degree all the disadvantages, such as the attendant hazards of fire and explosion.

Further objects of my invention are to produce an expansion joint material which is readily compressible, has a high degree of recovery, is non-extruding, and is resistant to the elements, moisture, etc.

In preparing my improved expansion joint, there is preferably first formed a vegetable fiber-board, composed of finely comminuted vegetable fibers suitably felted together to form the board. This board may be either formed independently or I may use certain forms of fiberboard already on the market, provided the same answer the requirements, as hereinafter set forth.

In the formation of this board, when the fibers are felted, there are formed or left between the fibers, small interstices or voids. The natural resiliency of the finely comminuted fiber itself, in

conjunction with these voids lends to the board a certain resiliency so that when compressed it will have an expansible action when the pressure is relieved therefrom. Thus the board so formed provides an admirable material in itself for use as an expansion joint in the respects above discussed. The density of the expansion joint material is preferably 0.235, however, it is within the scope of my invention that my novel method of making expansion joints may also be used with expansion joint material having a density as low as 0.120. The preferred range of the density of the expansion joint material when using my novel method of making expansion joints and dependent upon the specific use to which the material is utilized is therefore substantially within the range of the density of 0.120 to 0.270. However, I do not wish to limit myself to this specific range of densities for expansion joint material, but I would like to use my novel method with all suitable types and densities of felted fibers on the market or to be developed within the future.

It is obvious that the fiber board described above without being suitably treated would hardly be a suitable material for use in the respects noted for the reason that it might deteriorate when exposed to the elements, and also would be apt to readily absorb moisture, which would impair its resilient quality and also cause deterioration. I have found it necessary, therefore, in making use of this material to so treat it as to thoroughly incorporate therein preserving and waterproofing material. It is necessary, however, to so apply the preserving and waterproofing material that while it would substantially encase and somewhat impregnate the individual fibers of the mass it must not fill the interstices or air pockets in the mass of the board itself, since if the interfiber spaces or voids are filled the resiliency of the board is lost and its efficiency as an expansion joint largely destroyed.

I, therefore, accomplished the various objects of my invention by treatment of the board with the following materials and in the following manner:

The base material for the expansion joint material preferably comprises a relatively coarse fiber structural unit such as is available on the market generally as fiber insulating board, and which is manufactured by a process involving felting of the fiber from a water suspension of the fiber. Insulating board material which is a felted fiber product manufactured from relatively coarse fibers derived from vegetative sources contains a large proportion of interfiber air space

provided by the relatively loose fiber structure thereof, which characteristic imparts to the fiber sheet an appreciable resiliency and relatively high heat insulating value.

To prepare the base material for my novel expansion joint material and for the particular purposes of this invention, the sheet is first partially permeated or saturated with an asphaltic substance or with some other substance or compound having approximately the same general characteristics. The saturant should be relatively firm at ordinary temperatures such as are encountered in building constructions but should not be brittle and could well comprise an appropriate pitch or the like.

The saturant may be forced either by vacuum or by pressure treatment or by a combination thereof into and throughout the sheet material, however, in applying the saturant I prefer to use a dipping vat. The application of this saturant to the base material of the expansion joint should preferably be such that the fibers themselves are substantially coated and more or less saturated and a large part of, or substantially all of the interfiber or interior interstices or voids within the sheet are largely free of the saturating materials.

The saturant may be applied in any desired or convenient manner and instead of being driven into the materials by either vacuum, or pressure, or by a combination of such treatment, it may be applied by the submersion of the fiberboard in the saturant while such saturant is in a liquid state as by being maintained at an elevated temperature such that the saturant is liquid, or the saturant may be applied as a solution preferably of asphaltum and a light petroleum oil. Should it be preferable, it is to be understood that the base material for the expansion joint material might have incorporated therein during its process of manufacture sufficient of the asphaltic or other saturating substance whereby the fibers of the base material are substantially coated and are firmly bound together, which last method of preparation would involve a hot compression of the fiber sheet having the saturant distributed therethrough in order that the final product might be of a sufficient compactness, with the saturant thoroughly distributed over the fibrous surfaces thereof, due to the compression at elevated temperatures.

For the saturation or permeation of a fiber insulating board such as Celotex cane fiber insulating board of a density of substantially 0.235 or within the range of densities of fiberboard ranging from substantially 0.120 to 0.270, the preferred saturant is a Venezuelan residual asphalt of substantially the following characteristics:

100°-110° F. melting point, ring and ball, A. S. T. M. method.

180-200 mm. Pen. 100 g. 5 sec. 77° F. A. S. T. M. method.

525°-550° F. flash point Pensky Martens closed cup.

1.015-1.02 specific gravity.

25 sec. furol viscosity @ 375° F.

18 sec. furol viscosity @ 400° F.

The above asphalt is heated to a temperature preferably from 360° to 390° F. and the fiberboard or base material for the expansion joint material is immersed therein, and on being held so immersed for a period of time so that the fiberboard will absorb the described asphalt to the extent of substantially 100% based on the dry

weight of the fiberboard prior to immersion. In my preferred method, I desire that the saturant shall have only penetrated substantially a short distance from the surface of the fiberboard during the dipping operation and that this saturant shall be distributed throughout the fiberboard as will be described later.

While the preferred saturant has been described, it is to be understood that in the same general manner other saturants can be incorporated into the fiberboard and generally speaking any asphalt having viscosity not exceeding 30 sec. furol at 375° F. may be considered suitable providing, of course, it is raised to an appropriate temperature and that the fiberboard is held in such heated asphalt for a period of time sufficient, as may be necessary, to obtain the desired percentage of saturation. Among such asphalts are those made from petroleum cracking still residues (pressure tar pitches) which at 140° F. melting point will not exceed the viscosity just above stated. Blends of pressure tar pitches may be used with various residual asphalts of high melting point and high viscosity providing that the combination is such that the resulting viscosity falls within the limits of the viscosity above given. Still other saturants such as equivalent coal tars and oil tar pitches and blends may be used for saturation.

It is also within the scope of my invention that I may use a dipping bath composed preferably of asphaltum, and a flux, preferably a light petroleum oil. A suitable light petroleum oil which I prefer to use is known as Bunker "C" fuel oil having the following specifications:

|                        |                   |
|------------------------|-------------------|
| Gravity                | 14 A. P. I.       |
| Furol viscosity        | 122 @ 60° F.      |
| Pour point             | 40° F.            |
| Carbon residue         | Not to exceed 9%  |
| B. S. & W.             | Not to exceed .8% |
| Sediment by extraction | .5%               |
| Water by distillation  | 1 1/2%            |

I preferably use these with a portion thereof of each constituent so that the resultant saturant will readily penetrate the fiberboard. I heat the asphaltum to a fluid state and then add the oil. When the same are thoroughly mixed and in a perfect fluid state, and maintaining the same well heated, I immerse the fiberboard therein and allow it to remain in the bath a sufficient length of time for the fiberboard to be saturated from the surface thereof a definite distance, preferably 1/8", or for such a period of time that the fiberboard is impregnated from its surfaces inwardly with the solution, fluid, or saturant to the extent that the asphaltic contents of the finished board will vary from substantially 45% to 65% by weight of the finished board.

I have also found that it is possible to use a felted fiberboard having a density of 0.200 within a few hours of the time that the felted fiberboard has been made on the machine and dried, that is to say, it would be still dry and warm at the time of dipping. It is obvious that the time of dipping necessary to give a satisfactory penetration is dependent upon the density of the felted fiberboard. Using a standard saturant such as I have described, it has been found that a dipping time of from 15 to substantially 30 seconds in the saturant at a temperature of substantially 380° F. gave satisfactory results for 1/2" 0.200 density felted fiberboard. During this time the asphalt penetrated immediately to a depth of substantially 1/8" at each surface, and an asphalt up-

take of approximately 100% of the original weight of the board is obtained. I prefer to use dipping equipment comprising racks in which the boards are placed horizontally and dipped into the hot bath with a crane or other suitable apparatus. It is also within the scope of my invention that the felted fiberboard may be fed continuously through the hot asphalt or other saturant in order to effect the necessary uptake and penetration.

Although so far the description has been particularly with respect to  $\frac{1}{2}$ " material, I have found that felted fiberboard material of various thicknesses can be satisfactorily treated by my process. When using a thicker material it is preferable to use a lower density felted fiberboard, preferably having a density of not over 0.200 and have the board as dry and warm as practical before dipping. However, with my process I have been able to suitably saturate felted fiberboards which are substantially room temperatures. Higher density boards or boards that are not dry or which may have become cool before dipping require longer dipping time. In general, I have found that the  $\frac{1}{2}$ " felted fiberboard requires substantially a 5 second dip,  $\frac{3}{4}$ " board a 30 second dip, and 1" felted fiberboard substantially 2 minutes. The asphaltic content of the finished board used for expansion joint material will vary from substantially 45% to 65% by weight of the board.

After the felted fiberboards are removed from the dipping bath, the excess of saturant is preferably wiped therefrom by scraping or squeezing with rolls. The partly impregnated felted fiberboard partly saturated, inwardly from its surfaces, is then heated or baked to secure suitable penetration of the saturant throughout the board or sheet. To effect the necessary penetration I prefer to use hot stacks in place of an oven or direct heating of the felted fiber materials. With the hot stack method, the heat picked up by the felted fiberboard during the dipping process is utilized. In using this method, I prefer to use a hot dry board although it is obvious that a board at room temperature may be used. In using this method it is necessary to use a sufficiently fluid mixture of asphalt and oil and/or a suitable saturant to obtain complete penetration.

The felted fiber material after it leaves the apparatus for removing the excess saturant is close piled in a stack for several days. By this treatment due to the effect of heat and lapse of time, the saturant will distribute itself substantially uniformly throughout the felted material, at least to a point where there is substantially no unsaturated material showing when a sample is broken. It is preferable to suitably insulate the stack, and preferably the edges thereof, as by covering it with a heat insulation material to prevent heat losses therefrom. If it is necessary to maintain the required temperature of the hot stack, heat may be suitably supplied thereto. This process is called "dog-housing." The felted fiberboards are left in the hot stacks for substantially twenty-four hours more or less, or until the penetration or dispersion of asphalt or other saturant as disclosed is substantially complete, and the boards are then placed in cooling racks until sufficiently cooled to be repiled. Although I have disclosed the time for hot stacking as substantially twenty-four hours, it is within the scope of my invention that the felted fiber material may be hot stacked for a period of time necessary to obtain the penetration necessary or to obtain the characteristics

desired for the use to which the felted fiber material treated by my process is to be utilized.

Although I prefer to flat pile the felted fiber material, after it has been removed from the dipping bath in the hot stacks, it is also within the scope of my invention that the dipped board when stacked and piled may be stacked on edge. It is preferable in piling the board, that the edges or surfaces that were down in the dipping vat shall be uppermost in the hot stack.

The preferred characteristics of the expansion joint material formed and processed as described above are, a resiliency of not less than substantially 70%, a twenty-four hour water absorption not exceeding 12%, per cent asphalt by extraction within the range of substantially 45% to 65%, and substantially no odor. It should also be adapted to suitably bond to concrete. The test for resiliency is preferably determined on a sample 4" x 5" by compressing it to one-half its original thickness five times, allowing an interval of 90 seconds between pressing and 30 seconds under pressure. The ratio of the final expanded thickness taken one hour after the last pressing to the original thickness is the percent resiliency when multiplied by 100. It is preferable that the loss of weight should not be over 2%. The weight of the sample is taken before and after the resiliency test and the loss expressed as percent of original weight. The pressure for compression should preferably not be over 425 lbs. per square inch. In the foregoing specification of preferred characteristics, the compression pressure was substantially 140 lbs. per square inch. It is also preferable that the expansion joint material shall show no tendency to delaminate or disintegrate when given the hydrochloric acid test. For convenience in handling the finished expansion joint material, it should not be sticky.

By my novel method of substantially impregnating surface portions of the felted fiber material and then by heating, baking, or preferably by hot stacking, causing the impregnating substance to disperse or penetrate throughout the fiber material, I am able to suitably impregnate into and around the individual fibers of the mass, the asphaltum, the asphaltum and oil, or other suitable saturants. The hot stacking of the partially impregnated felted fiberboard by bringing about the dispersion of the saturant leaves the interstices or air voids in the board substantially unimpaired, so that the resiliency of the board is still present, although the fiber of the material is thoroughly waterproofed and preserved against deterioration. When a saturant of asphaltum and light oil is used, the light oil remaining with the asphaltum tends to keep the asphaltum in the mass in a softened condition rather than allowing it to become dry and hard, which might cause it to become brittle and breakable in use.

The material thus formed may be readily handled and cut up into various sizes and shapes for use as expansion joint material, due to its being in board form and readily capable of being cut, and handled at will; and, it has an inherent stability so that when placed in position it will remain intact without any tendency to slump or deform as is the common objection to certain other types of expansion joints.

From the foregoing description, it will be readily seen that I have produced a material for use as an expansion joint which has all the advantages necessary and none of the disadvantages referred to.

Now I have herein set forth the preferred

materials used in the construction of the joint, it is to be understood that I do not wish to limit myself to the use of any particular type of vegetable fiber or any particular waterproofing and preserving materials, the above being recited merely as the preferred material desired to be used in this regard, although in actual practice I would, of course, reserve the right to use any and all equivalent materials capable of the same use.

Having thus described my invention, what I claim as new and useful and desire to secure by Letters Patent is:

1. The method of treating a felted fiber board which comprises establishing a hot dipping bath of an asphaltic saturant, immersing fiber board in the bath and substantially impregnating the fiber board with the saturant to a limited depth from the surfaces thereof not exceeding one-fourth of the thickness of the felted fiber board, the fiber board removed from the bath and the saturant caused in part to migrate from the substantially saturated portion of the board into and throughout the unsaturated portion of the board by maintaining the board at an elevated temperature.

2. The method of treating a felted fiber board of substantially one-half inch to about one inch in thickness, and of a density of between 0.102 and 0.207 which comprises establishing a hot dipping bath of an asphaltic saturant maintained at the temperature of between about 360° F. to 390° F., immersing the fiber board in the bath for a time of from about thirty seconds to about two minutes and substantially impregnating the fiber

board with the saturant in the amount of from about 45% to 100% of the weight of the dry fiber board being treated, but to only a limited depth from the surfaces thereof, the fiber board removed from the bath and any excess saturant removed from the surface thereof, the saturant contained in the substantially saturated portion of the board caused to be distributed substantially uniformly throughout the entire board by holding the board at a temperature about that of the temperature of dipping.

3. The method of treating a felted fiber board as defined in claim 1, wherein the limited impregnation of the fiber board involves the addition to the board of the asphaltic saturant to the extent of from between about 45% to 100% of the dry weight of the fiber board.

4. The method of treating a felted fiber board as defined in claim 1 and wherein the asphaltic saturant is composed of asphalt and a flux oil.

5. As a new article of manufacture, a product produced in accordance with the method of claim 1.

6. As a new article of manufacture, a product produced in accordance with the method of claim 1, having a resiliency of not substantially less than 70%, a twenty-four hour water absorption not substantially in excess of 12%, and containing asphalt by extraction not in excess of 100%, but preferably in the amount of between about 45% to 65%, the product having substantially no odor.

CLARENCE R. ECKERT.